

May 9, 1944.

H. L. REED

2,348,360

## METHOD OF RECOVERING MINERALS

Filed Jan. 22, 1941



## UNITED STATES PATENT OFFICE

2,348,360

## METHOD OF RECOVERING MINERALS

Howard L. Reed, Austin, Tex.

Application January 22, 1941, Serial No. 375,441

16 Claims. (CL. 75—2)

This invention relates to the recovery of semi-metallic substances from their ores or from other mixtures and has for its general object the recovery of minerals from ores and the like, whether or not such aggregates contain large percentages of other substances which interfere with standard methods of metallurgical concentration. By the term "semi-metallic" I mean the group of elements including copper, bismuth, mercury, tin, antimony and arsenic.

This application is in part a continuation of my prior pending application Serial No. 342,075 filed June 24, 1940.

In another co-pending patent application Serial No. 342,127 filed June 24, 1940, I have described and claimed a method of recovering minerals from their ores, which consists of first sulphidizing the minerals to be recovered and then separating the sulphidized minerals from the gangue by various metallurgical processes, preferably by flotation. This unique process of treating crude ores with molten sulphur has been found extremely desirable for many types of ores, particularly those which contain inappreciable values of non-basic, or semi-metallic, mineral constituents.

The development of an efficient method of economically extracting these semi-metallic minerals from complex ores or concentrates, however, represents a very necessary objective of the science of metallurgy. For example, losses exceeding thirty per cent (30%) of the assayed tin content of certain complex Bolivian crude ores occur during the preliminary concentration thereof, exclusive of the excessive slag losses characterizing the subsequent smelting of such tin concentrates. Moreover, most of these tin concentrates, as finally imported from Bolivia, contain less than forty per cent (40%) of tin.

The metallurgical refinement of crude antimony oxide mineral ores is similarly inefficient. For example, almost a half million tons of such ore, assaying over five per cent (5%) antimony, several million dollars worth of mined and crushed mineral, has been abandoned by one company at a certain mining district in Mexico, for lack of a feasible process of concentration.

In an investigation for the purpose of providing a feasible process of metallurgical concentration, many crude ores were treated with molten sulphur. The basic oxide minerals were found to be readily altered to the corresponding metallic sulphides, respectively; and, thus sulphidized, were typically dissolved in the liquid sulphur medium and subsequently crystallized therefrom

when this solvent was evaporated. The sulphidized ore, thus dried of liquid sulphur, was then pulverized in a rod mill and discharged therefrom as an aqueous suspension of mineral slimes. 5 This product was thence fed to a flotation cell where the crystalline metallic sulphide particles were recovered by means of standard frothing reagents. These metallic, or basic, minerals were thus found to be readily sulphidized and efficiently extracted by means of the foregoing treatment, which effected a concentration ratio of forty to one in the case of copper oxide or copper carbonate crude ores; that is, the first flotation concentrate, the so-called rough concentrate, was 10 forty times as rich in copper as the tailings.

However, certain minerals, particularly the non-basic, or semi-metallic, minerals, of which the native oxides of antimony and tin are notable examples, have a tendency to chemically combine not only with the sulphur medium, during the vaporization thereof, but also with the limestone or other interfering basic, or metallic, substances which are frequently present in large amounts as constituents of the gangue material. Even in the absence of these interfering basic substances, the sulphidation of the semi-metallic oxide minerals by means of molten sulphur normally proceeds very slowly, in comparison with the rapid chemical alteration of the metallic oxide minerals by the molten sulphur medium. 20

In the case of certain Mexican antimony oxide mineral deposits, for example, such limestone represents about seventy per cent (70%) of the ore. 25 The interfering product formed by this reaction between the limestone and the sulphidized mineral is a calcium ortho-sulpho-antimonate



30 produced in various proportions with the primary alteration product, antimony sulphide,  $\text{Sb}_2\text{S}_3$ , and several secondary products such as calcium sulpho-antimonite,  $\text{Ca}_3(\text{SbS}_3)_2$ . These calcium compounds may be collectively termed the complex compounds of antimony sulphide with calcium sulphide, i. e.,  $(3\text{CaS})(\text{Sb}_2\text{S}_3)$  and  $(3\text{CaS})(\text{Sb}_2\text{S}_3)_2$ , etc. These complex secondary products have been considered objectionable since they are floated with some difficulty and since the mineral concentrate thus produced has a relatively small content of antimony, say forty per cent (40%), e. g., the calcium sulphide, combined as above with some of the antimony sulphide, tends to reduce the concentration. The 35 proportion of such calcium sulphide may be low-

ered by performing the sulphidization of the native ore at minimum temperatures, below the boiling point of sulphur; and by evaporating the excess sulphur at minimum temperatures, such as five hundred degrees centigrade; but the latter vaporization temperature does not allow rapid vaporization unless the particles of ore are relatively coarse, that is, larger than one eighth inch in diameter; whereas, rapid vaporization and minimum temperatures are essential for the prevention of calcification of the antimony sulphide. This practice has been employed and the above concentration thus made possible after the dried sulphidized ore has been ground in a rod mill to minus one hundred mesh and then floated. In other experiments the complex calcium antimony sulphides were partially dissociated by adding carbon dioxide to the water in the rod mill, during the pulverization of the sulphidized ore, such carbon dioxide being supplied under pressure by dry ice; and by employing carbon dioxide gas, rather than air, as a source of froth, when injected by the rotor into the flotation cell. A small increase in the antimony content of the flotation concentrate may thus be obtained; but the results are insufficient to provide a real solution to the problem. This problem of concentration of antimony oxide ores is a very important one because it has not been solved by any prior standard method of metallurgical refining.

It is an object of this invention, therefore, to eliminate the formation of the complex semi-metallic sulphides of calcium during the process of sulphidization.

Another object is to accelerate the sulphidization of the semi-metallic minerals.

It is a further object to provide a continuous process in which the sulphidizing medium will produce a single product; and to provide a process in which such sulphidized product will be readily soluble in water so that it may be more readily removed from the gangue.

It is a further object to provide a method whereby the dissolved sulphides of the semi-metallic elements may be recovered by flotation.

In order that the invention may be readily understood, reference is had to the accompanying drawing, forming a part of this specification, and in which the single figure is in the nature of a diagram or flow sheet illustrating an ore crusher, rotary kiln, rod mill, flotation cells, etc., used in carrying out the invention, and showing the relation of these various pieces of apparatus to each other. In this drawing, I have indicated optional steps or the optional addition of certain materials by dotted or broken arrows.

I have discovered that the formation of the complex semi-metallic sulphides of calcium may be inhibited during the sulphidization process and that the sulphidization process may be greatly accelerated by the previous introduction into the ore of material containing another or other elements which will combine with the sulphidized mineral much more readily and quickly than will the calcium. Numerous such materials may be employed. One such material, which has been found very suitable, is sodium carbonate. Certain non-alkaline compounds of sodium or potassium would also serve this purpose.

As an example of the use of sodium carbonate, a crude antimony oxide ore having a relatively large proportion of limestone was pulverized and mixed dry with an equal weight of flowers of sulphur and with a relatively small amount of

sodium carbonate, about one part of the latter to ten parts of sulphur. This mixture was heated rapidly and the excess sulphur vaporized. The residue was then leached with plain water by

5 boiling the latter with the residue. The solution was filtered and thence injected with hydrogen sulphide gas, which decomposed the dissolved sodium thioantimonate and thus precipitated antimony penta-sulphide, which was thence recovered 10 by filtration.

In large scale operations, the aqueous filtrate obtained from the filtered residue may be injected into a gas and liquid contact apparatus with the gases produced during the sulphidization of the crude ore.

This causes a precipitation of antimony penta-sulphide uncontaminated with other products of sulphidization, this antimony sulphide being seventy-one per cent (71%) antimony by weight.

20 The precipitation of this antimony sulphide is effected by the injection of the discharge flue gas from the rotary kiln where the ore is first treated, which flue gas consists of carbon dioxide produced by the combustion of the fuel and also of sulphur dioxide produced by the sulphidization of the oxide minerals in the kiln. Both gases, when injected into the aqueous filtrate, acidify this solution of the complex sulphidization products of sodium and produce insoluble antimony

25 sulphide and soluble sodium thiosulphate by the preliminary neutralization of the excess alkali and by the decomposition of the complex semi-metallic sulphides of sodium:



In my previous application Serial No. 342,075 it was stated that sodium carbonate and sodium 40 sulphite are also produced; but I have found that if these latter substances are produced they will both be immediately attacked by the sulphur dioxide gas and thus altered to sodium thiosulphate.

I have discovered that this sodium thiosulphate 45 may be re-used as a part of the charge with the crude ore and sulphur at the beginning of the process. Such use of this non-alkaline compound of sodium is thus an important feature of this invention for by virtue thereof the process becomes continuous; and by virtue thereof the necessity for the consumption of sodium derived from an outside source is practically eliminated, whereas, if sodium carbonate were to be employed alone, as in the initial phase of this process, the silicious gangue would be attacked thereby and altered to sodium silicate:



Accordingly, the demineralized aqueous solution of regenerated sodium thiosulphate may be continuously returned to the rotary kiln, wherein the water solvent will be quickly evaporated as the crude ore mixture is heated.

The gradual progress of this crude charge toward the interior of the slightly inclined, slowly rotating, cylindrical kiln is attended by increasing temperatures and by the spontaneous thermal decomposition of the sodium thiosulphate into sodium sulphate and molten penta-sulphide 65 of sodium. The latter dissolves energetically in the liquid sulphur, which forms an ideal fusion medium with the sodium sulphate.

This alkalinized sulphur medium, generated and maintained within the rotary kiln, vigorously attacks the oxide minerals submerged therein by

reducing them to sulphides, with the evolution of sulphur dioxide, and by simultaneously neutralizing such sulphides while producing the soluble complex sulphidization products of sodium:



During the sulphidization of these oxide minerals, however, the limestone gangue remains undecomposed; whereas, in the absence of dissolved sodium penta-sulphide, a much higher temperature would be required for the chemical decomposition of the semi-metallic oxides by molten sulphur alone, in which case both the limestone and the antimony oxide would be jointly sulphidized and compounded as the sulpho-antimonate of calcium:



The continuous consumption of sodium penta-sulphide, during the sulphidization of the oxide minerals, is continuously compensated by the regeneration of additional sodium penta-sulphide, as performed by the spontaneous thermal decomposition of the sodium thiosulphate, as delivered to the kiln by the demineralized liquor:



Additional sodium penta-sulphide is reproduced by the sulphidization of a certain portion of the sodium sulphate formed by the foregoing decomposition reaction. This sodium sulphate tends to be reduced, by molten sulphur, to sodium sulphite. This preliminary product is unstable at these temperatures; hence the sodium sulphite experiences spontaneous thermal decomposition, thus creating sodium sulphate and sodium sulphide. The latter product immediately reacts with molten sulphur, thus regenerating additional sodium penta-sulphide:



The chemical equilibrium of the foregoing reaction maintains a constant concentration of dissolved penta-sulphide of sodium in the molten sulphur medium. This equilibrium tends to be disturbed, of course, by the consumption of this alkali by the semi-metallic minerals; but such consumption is continuously compensated by the above phenomena of chemical regeneration of additional penta-sulphide of sodium. Consequently, the sodium sulphate regenerator must be considered as the primary sulphidizing reagent, in view of the fact that this salt constitutes the only source of sodium penta-sulphide which can maintain the chemical equilibrium of these kiln reactions.

By virtue of this process numerous economies are effected. The first which is apparent, is that the first phase of the process, namely the reactions of the various materials within the kiln, produces gases which are employed to cause the precipitation of the antimony sulphide at the end of the process. Thus the necessity for providing any separate source of reagent for causing this precipitation is eliminated and great economy results therefrom.

Second, the result of the reaction during the precipitation of this antimony sulphide is a non-

alkaline barren liquor which contains sodium thiosulphate; and this liquor is used in forming the charge for the kiln in the first step of the process so as to provide the sodium and a portion of the sulphur required for continuously charging the kiln. Thus the sodium is re-used again and again and the cost of sodium sulphate, or other source of sodium, such as sodium thiosulphate, sodium sulphide or sodium carbonate,

is limited to the cost of such amounts as are necessary to replace leakage and unavoidable waste.

At the same time, the use of this demineralized sodium thiosulphate liquor cuts down the necessary amount of sulphur for the charge to the

15 rotary kiln.

In addition to the economies just mentioned, the elimination of waste products avoids the necessity of providing for the disposition of such products and provides a continuous process, which is highly useful and advantageous commercially.

It is also to be noted that this process conserves heat because whereas sodium carbonate has a melting point of substantially 850° C., sulphur has a melting point of 120° C. and a boiling point of 445° C., approximately. The sodium penta-sulphide, which fuses at 252° C., forms a fusion medium with molten sulphur and sodium sulphate which will very quickly react with the antimony oxide or tin oxide, or other semi-metallic minerals, at a temperature below 445° C.; whereas, in the absence of such alkalinized sulphur, a temperature of 850° C. would be required to produce a water soluble antimony compound by means of sodium carbonate. Moreover, the excess sodium carbonate could not be retained in the kiln; whereas, the excess sulphur is automatically evaporated and refluxed and re-condensed therein, thus conserving both heat and sulphur. Finally, the heat required to melt, boil and vaporize sulphur is approximately one fourth of that required to convert ice into steam.

The sulphidization equipment for the process described may be broadly similar to that employed for the calcination of limestone, and is diagrammatically shown in the accompanying drawing.

The demineralized liquor will be fed to this rotary kiln, which is also fed continuously with the crude crushed ore and sulphur. The products from the rotary kiln are discharged into a rotary cooler and thence preferably fed to a rod mill, or the equivalent, and thence to any suitable filtering or separating apparatus where the solution may be separated from the insoluble tailings. This aqueous filtrate is then delivered to any suitable gas and liquid contact apparatus in the presence of the exhaust gases from the intake end of the rotary kiln, thus causing the precipitation of the antimony sulphide, or other semi-metallic sulphide, as above described. These precipitated sulphides may then be separated from the barren liquor by filtration or by any other suitable process.

65 It will be understood that the limestone above referred to is only one example of a number of substances which might constitute the interfering constituents of an ore. In the case of tin ore, for example, it is frequently found that 70 quantities of iron oxide are present with the tin oxide; and that the iron oxide acts as an interfering substance in that it possesses characteristics which cause it to be recovered with the tin oxide if any standard method of concentration is employed.

The use of an alkalinized sulphidizing medium in accordance with this invention makes possible the recovery of tin from such ore without interference from the iron oxide or similar basic compound because it causes the formation of a water soluble compound of tin, just as in the previous example a soluble compound of antimony was formed. Just as the limestone in the previous example emerges from the kiln in the form of an insoluble compound, so in this instance the iron would likewise emerge from the kiln in the form of an insoluble compound. The tin, in the form of thio-stannate of sodium, may then, of course, be removed by leaching the sulphidized ore with water, as in the case of the antimony. Any of the various metallic oxides, or other basic compounds, present as a part of a semi-metallic ore would behave in a similar manner and be discharged from the kiln as insoluble products of sulphidization.

If such tin or antimony or other semi-metallic ore require the segregation of several semi-metallic constituents or the individual extraction of the metallic constituents, then, in this event, the foregoing process may be readily extended toward the realization of these objectives.

Accordingly, the metallurgical refinement of complex minerals in general, and of the Bolivian tin concentrates in particular, justified the further development of this process, since commercial quantities of copper and silver, as well as the tin content thereof, must be separately recovered from the ferrous gangue.

As in the introductory problem of calcareous antimony oxide ores, the alkalinized sulphur medium performs the chemical decomposition and preliminary sulphidization of these crude complex ores, such as the Bolivian tin oxide minerals.

This refractory crushed ore is fed to the cooler end of a rotary kiln, which is inclined toward its outlet end, having an annular partition or ring located below the mid-portion thereof. The complex ore is automatically mixed with a saturated aqueous solution of sodium thiosulphate during its continuous progress along the slightly inclined, slowly rotating, cylindrical kiln. Sulphur may or may not be added with this charge, the addition of sulphur being made unnecessary by the fact that sufficient sulphur is provided from the decomposition of the sodium thiosulphate to permit the carrying out of the process. The translation of this raw mixture is attended by the evaporation of the entrained water during the preheating thereof by a counter-current of kiln gases. The slow and gradual descent of this mineralized charge toward a central reservoir of alkalinized molten sulphur, retained by said annular partition, is thus characterized by increasing temperatures and by the increasing condensation of sulphur vapor thereupon. Heat and sulphur are thus continuously absorbed by the advancing charge. Steel ribs, or lifting flights, may, if desired, be secured to the interior surface of the revolving cylindrical shell, axially parallel to the spiralized motion imparted to the ore, in order to promote an efficient heat exchange between the ore thus distributed and the counter-current of hot kiln gases.

The passage of this mineralized charge through the preheating zone of the rotary kiln witnesses the spontaneous thermal decomposition of the entrained sodium thiosulphate into sodium sulphate and sodium penta-sulphide, as well as the rapid fusion of the latter.

The arrival of the preheated crude ore at the

surface of the liquid sulphur medium is attended by the dissolution of the entrained molten sodium penta-sulphide. During the continuous progress of the complex minerals through the

alkalinized sulphur medium, their chemical decomposition is accelerated by the complete dissemination of the ore particles submerged in this turbulent medium, agitated by the action of the steel ribs, which promote an intimate diffusion of the mineral constituents with the dissolved sodium penta-sulphide.

The gradual descent of this sulphidizing charge through the shallow reservoir of agitated liquid sulphur is further characterized by the evolution of sulphur dioxide which is thence conveyed by the kiln gas toward the cooler end of the rotating kiln where these gaseous products are received by an aspirator.

The chemical transformation of the basic oxide minerals into the corresponding metallic sulphides, and of the semi-metallic minerals into the corresponding complex semi-metallic sulphides of sodium, identifies the character of the sulphidized products which, together with the inert calcareous or siliceous gangue material, finally arrive at the foot of the shallow sulphur reservoir where they are impeded by the steel ring which interrupts their gradual descent through the rotary kiln.

These products of sulphidization, submerged in the molten sulphur medium, are thus temporarily impounded by a transverse circular dam, in effect, over which they continuously spill as they are lifted from the alkalinized sulphur reservoir by the action of the steel ribs secured to the interior surface of the slowly revolving cylindrical kiln. A portion of the liquid sulphur is conveyed by the ore which overflows this annular dam into the evaporation zone of the rotary kiln.

During the progress of this mixture of sulphidized ore and alkali saturated sulphur toward the lower end of the kiln, the increasing temperature accelerates the evaporation of the entrained boiling sulphur. The distillation of this solvent, which is saturated with the dissolved products of sulphidization and particularly charged with sodium penta-sulphide, produces a liquid residuum of the latter molten alkali which retains in solution the various metallic sulphides and complex semi-metallic sulphides of sodium. The sulphur vapor which distills from this sodium penta-sulphide residuum is conveyed, of course, by the counter-current of kiln gas toward the cooler zones of the kiln, where this refluxing sulphur vapor condenses upon the approaching charge of raw complex ore, crude sulphur and sodium thiosulphate brine.

The foregoing liquid residuum as well as any products of crystallization, including minor amounts of sodium sulphate, are finally discharged with the inert gangue material from the lower end of the rotating kiln.

This unsintered aggregate of kiln products, dried of liquid sulphur, is received by an inclined, cylindrical, rotary cooler, wherein oxidation of the hot material is prevented by exclusion of air, which delivers them into a hopper which feeds the rotating trunnion of a standard rod or ball mill. The latter is fed, of course, with water also; but only an absolute minimum thereof, since it is essential that the maximum concentration of dissolved penta-sulphide of sodium be continuously maintained during such aqueous dilution, which immediately precipitates the insoluble metallic or basic sulphides, in order to pre-

vent the precipitation of the appreciably soluble sulphides of copper and bismuth.

This requirement of maximum concentration of dissolved alkali necessitates the continuous maintenance of a temperature exceeding 90° C., during the pulverization and subsequent treatment of these hot kiln products. This maximum concentration of dissolved alkali may preferably be determined and indicated by a standard pH meter.

The hot pulverized material, thus super-saturated with sodium penta-sulphide, is discharged from the rod mill into a standard classifier, which delivers the usual aqueous suspension of slimes, whereas the coarser particles which settle therefrom are automatically returned to the rod mill.

This hot aqueous suspension may be conducted to a primary series of flotation cells, where the insoluble metallic sulphides will be recovered.

This preliminary flotation of the sulphides of manganese, iron, cobalt, nickel, zinc, cadmium, silver and lead, which are herein referred to as metallic, or basic, sulphides, will be performed in accordance with the standard methods of flotation procedure, except that, for reasons which will be hereinafter stated, the usual metallic sulphide froth will be produced in these cells by the injection of steam, rather than air, through the respective rotors thereof. The froth which overflows from this series of cells may be treated for the selective flotation of the valuable constituents or followed by the cyanidation of the silver sulphide. The customary operations of settling and thickening will recover the excess liquor, which may be returned to the slime suspension discharged as tailings from the preliminary flotation stage.

This hot aqueous suspension of gangue particles may now be circulated through a standard automatic filter in order to reject such gangue material from the mineralized filtrate.

An analysis of this hot mineralized filtrate containing the so-called soluble sulphides of the semi-metallic elements, will indicate the principle by virtue of which the mineral solute may be selectively extracted, in view of the respective characteristics of four types of dissolved constituents, which may be identified and classified as follows:

(1) The non-mineralized sodium compounds, e. g., sodium sulphate and sodium penta-sulphide; and

(2) Those mineral sulphides which are merely soluble by virtue of the maximum concentration of dissolved sodium penta-sulphide, e. g., copper and bismuth sulphides; or further dependent for such solubility upon the presence of tin sulphide, as is the prerequisite in the case of the dissolved copper sulphide; and

(3) Those complex semi-metallic sulphides of sodium which are soluble in an aqueous solution of sodium thiosulphate and sodium sulphate by virtue of a limited or partial concentration of dissolved sodium penta-sulphide, i. e., the sulphides of mercury and tin; and

(4) Those complex semi-metallic sulphides of sodium which remain dissolved in a neutralized aqueous solution of sodium thiosulphate and sodium sulphate, in spite of the absence of sodium penta-sulphide, i. e., sodium thioantimonate and sodium thio-arsenate.

Accordingly, this hot complex aqueous filtrate may be conducted to a second series of flotation cells, actually a system of several parallel series of cells, where the second group of mineral sul-

phides, copper and bismuth, will be successively precipitated and extracted with the froth produced in these cells by the usual injection of air through the respective rotors thereof.

During the continuous progress of the hot mineralized filtrate through any single series of these secondary cells, the gradual and cumulative decomposition of the dissolved sodium penta-sulphide will be performed by the oxygen content of the air injected therein:



This production of sodium thiosulphate, a very soluble non-alkaline salt, attends the destruction of a portion of the dissolved alkali, sodium penta-sulphide. Moreover, since maximum concentration of the latter was required to maintain in solution therewith the sulphides of copper and bismuth, it is impossible to prevent the precipitation of these dissolved sulphides except prior to the injection of air into this solution. It is for this reason that steam, rather than air, must be used in the preliminary flotation of the insoluble sulphides of the so-called metallic, or basic, elements, as heretofore mentioned.

The successive precipitation and hence the selective flotation of the dissolved sulphides of copper and bismuth, respectively, from a solution, as distinguished from the usual flotation of sulphides from a suspension, represents an efficient and continuous method of metallurgical concentration of these pure sulphides, uncontaminated with the usual proportion of silicious or calcareous gangue particles, thus revealing an ideal degree of flotation proficiency.

The semi-neutralized liquor discharged from the secondary flotation stage will be received by a third system of flotation cells, arranged in several parallel series, where the third group of mineral sulphides, mercury and tin, will be successively precipitated and extracted with the froth produced in these cells by the injection of kiln gas, through the respective rotors thereof.

During the continuous progress of the mineralized liquor through any single series of these third class cells, the cumulative decomposition of the dissolved penta-sulphide of sodium will be continued by, and finally completed by, the sulphur dioxide content of the kiln gas injection:



During this production of additional sodium thiosulphate, the complex semi-metallic sulphides of sodium are also attacked by the sulphur dioxide gas. For example, this chemical decomposition of the dissolved sodium thio-stannate produces the insoluble tin sulphide, as well as additional sodium thiosulphate:



The successive precipitation and hence the selective flotation of the sulphides of mercury and tin, respectively, represents a continuous method of metallurgical concentration of these pure sulphides by means of the simple expedient of simultaneous precipitation and flotation.

The froth which overflows from these third class cells will be settled and thickened as usual; whereas, the excess liquor thus obtained will be returned to the mineralized solution and hence will be discharged from this third flotation stage as a neutralized solution of sodium thiosulphate, sodium sulphate, sodium thioantimonate and sodium thioarsenate.

The final phase of demineralization of this neutralized liquor may be similarly performed in a

fourth system of flotation cells, wherein the sulphides of antimony and arsenic will be successively precipitated and hence selectively extracted with the froth produced therein, either by the injection of kiln gas or by the injection of concentrated sulphur dioxide. The latter may be obtained by condensation, if the kiln gases are circulated through a "gas separator" at a pressure of fifty pounds per sq. in.

During the continuous progress of this neutralized liquor through any single series of these fourth class cells, the cumulative decomposition of the dissolved thio-antimonate of sodium will be performed by the sulphur dioxide injection:



This precipitation and hence the flotation of antimony penta-sulphide is thus attended by the formation of additional sodium thiosulphate and, as usual, by the further conservation of the sulphur dioxide content of the kiln gas.

The subsequent decomposition of the dissolved sodium thio-arsenate and the consequent precipitation and flotation of arsenic penta-sulphide will be performed by the injection of both sulphur dioxide and steam, since a temperature of one hundred degrees centigrade is required during this final phase of demineralization of the aqueous liquor.

This continuous production of barren liquor may be delivered to the rotary kiln where this solution will serve as a primary source of sodium thiosulphate and sodium sulphate.

During the subsequent evaporation of this solution in the preheating zone of the rotary kiln, quantities of steam will be produced and thence aspirated therefrom, together with the flue gas.

These aspirated vapors will also contain a portion of the very volatile arsenic penta-sulphide, as produced by the thermal decomposition of sodium thio-arsenate during the distillation of the excess sulphur from the sulphidized ore and sodium penta-sulphide residuum, unless a sufficient excess of the latter solvent prevents such decomposition.

The recovery of the arsenic penta-sulphide may be accomplished by circulating these aspirated kiln gases through a condensation trap, wherein the entrained steam will be condensed and discharged therefrom as an aqueous suspension of arsenic penta-sulphide.

This condensate may also contain suspended sulphur which escaped from the preheating zone of the sulphidization kiln as a mist of sulphur dispersed in the kiln gas and thus was aspirated from the kiln. The specific recovery of this sulphur, as well as the suspended arsenic penta-sulphide, may be effected by circulating the condensate through two flotation units.

The extraction of this finely divided sulphur will be readily performed in the first of these units by the addition of a trace of pine oil to the aqueous suspension. This weak frothing reagent serves as a specific collector during this flotation of suspended sulphur.

The subsequent recovery of the arsenic penta-sulphide will be readily performed in the second of these flotation units by the addition of a trace of amyl xanthate to the aqueous suspension. This relatively stronger frothing reagent serves as a collector of any sulphidized mineral during the flotation thereof, either from the above condensate or from any of the mineralized media treated during the preceding phases of flotation.

The principal feature, therefore, of the foregoing method of refining the condensate is emphasized by the applicability of this principle to the various phases of this process, whereby the specific recovery of the sulphur, as precipitated during the neutralization of the sodium penta-sulphide, or during the decomposition of the complex semi-metallic sulphides of sodium, may be performed prior to the flotation of the precipitated mineral sulphides; whereas, the latter will thus remain in suspension until the secondary frothing reagent, as above, is added to the liquor arriving in the final section of any single series of flotation cells. The sulphur thus extracted will be settled and thickened as usual, of course, and thence returned to the rotary kiln.

This metallurgical process of continuously refining complex minerals by aqueous lixiviation and by selective flotation has produced individual concentrates of relatively pure sulphides of the semi-metallic elements. These sulphide products may be decomposed electrolytically, by virtue of their solubility, respectively, in a molten sulphur medium.

The significance of this final expedient may be appreciated by consideration of the difficulties which are usually encountered during the electrolysis of metallurgical products, such as the decomposition of the electrolyte. A molten sulphur electrolyte, however, can not be decomposed, of course. Moreover, this cheap medium has sufficient electrical resistivity to be maintained in a molten state by the conduction of the electrolytic current. Furthermore, this current may be regulated by the applied voltage, which will automatically control the temperature of the sulphur solvent. In particular, if this temperature corresponds to the boiling point of sulphur, 445° C., then, in this case, the excess sulphur produced by the electrolysis of the mineral solute may be continuously removed as vapor from the electrolytic cell and subsequently condensed. Finally, this operating temperature permits the continuous production of liquid metals, in the case of tin, bismuth, lead, cadmium, zinc and arsenic, during the electrolytic decomposition of their respective sulphides.

The objects hereinbefore expressed have thus been fully realized. The economical production of the individual concentrates of the semi-metallic sulphides, although characterized by flotation procedure, reveals the performance of an ideal function of the flotation process, whereby the respective mineral products have been selectively precipitated and simultaneously floated from the filtered solvent medium and thus efficiently refined to a degree not hitherto achieved. The cost of the entire metallurgical refining process has been found to be very low, being approximately one cent per pound of sulphidizable elements fed to the sulphidization kiln.

Having described my invention, I claim:

1. In a continuous method of recovering mineral values from a mass containing an element capable of forming a water-soluble alkali compound with sulphur, the steps of causing such mass to flow in a substantially continuous stream through zones of progressively increasing temperatures, mixing with such mass as it flows an excess of sulphur and an alkali, the temperature of the hottest of such zones being sufficient to cause a rapid sulphidization of said mass and vaporization of the excess sulphur, causing the sulphur vapor so produced to flow toward the cooler of said zones, and condense upon the

stream of material flowing toward the hotter of such zones, leaching with water the solid materials flowing from the hottest of such zones, drawing off the aqueous solution, treating said aqueous solution with the gases from said heated zones to cause the precipitation therefrom of the insoluble sulphide of said element, collecting the barren liquor after such precipitation and mixing it with the stream of material entering said heated zones.

2. In a method of recovering mineral values from a mass containing an element capable of forming a water-soluble alkali compound with sulphur, the steps of causing such mass to flow in a substantially continuous stream through zones of progressively increasing temperatures, mixing with such mass as it flows an excess of sulphur and an alkali, the temperature of the hottest of such zones being sufficient to cause rapid sulphidization of said mass and vaporization of the excess sulphur, causing the sulphur vapor so produced to flow toward the cooler of said zones and condense upon the stream of material flowing toward the hotter of such zones, leaching with water the solid materials flowing from the hottest of such zones, drawing off the aqueous solution, and acidifying said solution to cause the precipitation therefrom of the insoluble sulphide of said element.

3. In a method of recovering minerals from a mass of ore containing compounds of copper, bismuth, tin, mercury, antimony, arsenic and other elements, the steps of sulphidizing such ore in the presence of an alkali, leaching the sulphidized ore in a non-oxidizing atmosphere with an amount of water insufficient to dissolve all of the alkali in said sulphidized ore, adding a frothing agent, injecting steam into the resulting mass to produce flotation of insoluble metallic sulphides therefrom, filtering off the concentrated alkaline solution of the soluble sulphides, injecting air into said solution to cause the simultaneous precipitation and flotation of copper and bismuth sulphides from said solution, injecting sulphur dioxide into said solution to cause the simultaneous precipitation and flotation of tin and mercury sulphides from said solution, injecting additional sulphur dioxide into said solution to cause simultaneous precipitation and flotation of antimony sulphide from said solution, and injecting sulphur dioxide and steam into said solution to cause the simultaneous precipitation and flotation of arsenic sulphide therefrom.

4. In a method of recovering minerals from a mass of ore containing elements, some of which are capable of forming water-soluble alkali compounds with sulphur, and others which are not, the steps of sulphidizing such ore in the presence of an alkali, leaching the sulphidized ore with an amount of water insufficient to dissolve all of the alkali in said sulphidized ore, adding a frothing agent and injecting steam into the resulting mass to produce flotation of insoluble metallic sulphides therefrom without removing the soluble sulphides.

5. The method of recovering valuable constituents from a mass containing elements capable of forming water-soluble alkali sulpho-salts where such mass contains also interfering substances, which comprises sulphidizing the mass in the presence of an alkali to produce water soluble compounds, leaching the sulphidized mass with water to obtain a solution of such compounds, drawing off the solution, adding a frothing agent, and injecting into the solution an acidifying gas

to cause precipitation of insoluble sulphides and the simultaneous flotation thereof.

6. The method of recovering valuable constituents from a mass containing elements capable of forming water-soluble alkali sulpho-salts where such mass contains also interfering substances, which comprises sulphidizing the mass in the presence of an alkali to produce water soluble compounds, leaching the sulphidized mass with water to obtain a solution of such compounds, drawing off the solution, adding a frothing agent, and injecting acid kiln gas into the solution to cause precipitation of insoluble sulphides and the simultaneous flotation thereof.

15 7. The method of recovering valuable constituents from a mass containing elements capable of forming water-soluble alkali sulpho-salts where such mass contains also interfering substances, which comprises sulphidizing the mass in the presence of an alkali to produce water soluble compounds, leaching the sulphidized mass with water to obtain a solution of such compounds, drawing off the solution, adding a frothing agent, and injecting into the solution the gas resulting from the sulphidizing step to cause precipitation of insoluble sulphides and the simultaneous flotation thereof.

20 8. The method of recovering antimony from a mass containing antimony and limestone which comprises sulphidizing the mass in the presence of an alkali to produce a water soluble compound of antimony, leaching the sulphidized mass with water to obtain a solution of said compound, drawing off the solution, adding a frothing agent, and injecting an acidifying gas into the solution to cause simultaneous precipitation and flotation of the antimony sulphide therefrom.

25 9. The method of recovering tin from a mass containing the same where such mass contains iron oxide, which comprises sulphidizing the mass in the presence of an alkali to produce a water soluble compound of tin, leaching the sulphidized mass with water to obtain a solution of such compound, drawing off the solution, adding a frothing agent, and injecting an acidifying gas into the solution to cause simultaneous precipitation and flotation of the tin sulphide.

30 10. The method of recovering valuable constituents from substances containing an element 40 of the group consisting of antimony, tin and bismuth which involves treating such substances with sodium thiosulphate in the presence of molten sulphur and then leaching the product with water.

35 11. The continuous method of recovering mineral values from a mass containing an element 45 capable of forming water-soluble alkali sulpho-salts which involves treating such mass with sodium thiosulphate in the presence of molten sulphur, leaching the product with water, drawing off this aqueous solution and injecting the same with sulphur dioxide gas in order to precipitate the sulphide of such element and in order to regenerate sodium thiosulphate; and re-using this 50 non-alkaline compound to recover additional mineral values.

40 12. A continuous process for recovering mineral values from a mass containing an element 55 capable of forming a water soluble alkali sulpho-salt, which comprises heating said mass with an alkali in the presence of molten sulphur, dissolving the resulting alkali sulpho-salt out of the product, and adding sulphurous acid to the solution, whereby the insoluble sulphide is precipitated and alkali metal salts regenerated, and re-

using such alkali metal salts to mix with said mass during the heating step.

13. A continuous process for recovering mineral values from a mass containing an element capable of forming a water soluble alkali sulpho-salt, which comprises heating said mass with sodium thiosulphate, dissolving the resulting alkali sulpho-salt out of the product, and adding sulphurous acid to the solution, whereby the insoluble sulphide is precipitated and sodium thiosulphate regenerated.

14. A continuous process for recovering mineral values from a mass containing an element capable of forming a water soluble alkali sulpho-salt, which comprises heating said mass with sodium thiosulphate in the presence of other sodium compounds, dissolving the resulting sodium sulpho-salts out of the product, adding sulphurous acid to the solution in order to precipitate the insoluble sulphide and to regenerate sodium salts, including sodium thiosulphate, and re-using such regenerated sodium salts to mix with said mass during the heating step.

15. In a method of recovering minerals from a mass of ore containing elements, some of which

are capable of forming water-soluble alkali compounds with sulphur and others which are not, the steps of sulphidizing such ore in the presence of an alkali, treating the sulphidized ore with water, adding a frothing agent and injecting steam into the resulting mass to produce flotation of insoluble sulphidized compounds therefrom without removing the soluble sulphidized compounds.

16. In a method of recovering minerals from a mass of ore containing elements, some of which are capable of forming water-soluble alkali compounds with sulphur and others which are not, the steps of sulphidizing such ore in the presence of an alkali, treating the sulphidized ore with water, adding a frothing agent, injecting steam into the resulting mass to produce flotation of insoluble sulphidized compounds therefrom without removing the soluble sulphidized compounds, injecting an acidifying agent into the remaining solution to cause precipitation of soluble sulphides, and removing by filtration the precipitate thus formed.

HOWARD L. REED